

(No Model.)

E. M. THOMPSON.

ENAMELED WARE.

No. 355,486.

Patented Jan. 4, 1887.

Fig. 1.



Fig. 2.



WITNESSES.

Gustav Bohm.  
Hattie Kury.

INVENTOR.

Evert M. Thompson.  
By C. P. Jacobs  
atty.

# UNITED STATES PATENT OFFICE.

EVERT M. THOMPSON, OF EVANSVILLE, INDIANA.

## ENAMELED WARE.

SPECIFICATION forming part of Letters Patent No. 355,486, dated January 4, 1887.

Application filed July 21, 1886. Serial No. 208,662. (No model.)

*To all whom it may concern:*

Be it known that I, EVERET M. THOMPSON, a resident of Evansville, Indiana, have made certain new and useful Improvements in Enameled Wares, a description of which is set forth in the following specification, reference being made to the accompanying drawings, in the several figures of which like letters refer to like parts.

My invention relates to a new method of making enameled wares, either flat, round, or hollow; and it consists, substantially, in superimposing upon each side of a foundation composed of woven wire-cloth or perforated metal a suitable enamel, a portion of which will pass entirely through the interstices of the wire, uniting the enamel on both sides, and composing, substantially, a solid sheet or dish of enameled material. The wire foundation may be in a flat sheet, and in this condition, being covered with the enamel, may be formed into various articles of builders' use, such as shingles, gutters, and a variety of other articles, which are at the same time water-proof, rust-proof, and fire-proof.

In the drawings, Figure 1 represents a vase embodying my invention, a portion of the outside enamel, *e*, being broken away, showing the wire foundation *w* beneath. Fig. 2 is a vertical section of the same vase, showing the wire foundation centrally embedded in the enamel.

Heretofore enamel of various kinds has been deposited upon a sheet-metal base, generally iron, and the process commonly in use is as follows: The metal intended to be coated with enamel is covered with acid, which is then washed off and a coating of gum is applied, and a glaze which is in the form of a powder is then sifted over the gum, causing the powder to adhere to the metal base, and the articles are then placed in an oven or furnace and

heated until the glaze fuses and runs together, forming a continuous enameled surface over such portions of the sheet as have been covered with the powder. This process only puts an enameled coating over a solid base, and the latter under the action of heat and cold expands and contracts unequally with the enamel, causing it to crack and peel off. Instead of this solid base, I use the flexible wire foundation *w*, and the enamel may be either flexible or hard enamel, and the woven wire may be worked or stamped into a variety of articles for use—such as pails, pans, and cooking utensils—and after being modeled may then be enameled by my process. The sheet of wire may be treated in a similar manner to that indicated above and commonly used for the sheet-metal wares. The wire foundation is cleaned with acid, washed, and coated with gum, and the enamel is sifted on one side and then sifted upon the other, so as to entirely coat both sides of it, and then baked in a furnace until the glaze fuses, and it will run over both sides of the wire and through the openings, uniting the enamel at those points, and completely covering up the wire foundation, and the article will appear to be only made of the enamel itself, the wire foundation being completely concealed, as shown in the drawings hereto annexed.

What I claim as my invention, and desire to secure by Letters Patent, is the following:

As an article of manufacture, a vase or other article formed of enamel deposited upon a woven-wire foundation, substantially as and for the purpose described.

In witness whereof I have hereunto set my hand this 14th day of July, 1886.

EVERET M. THOMPSON.

Witnesses:

C. P. JACOBS,  
HATTIE MURRY.